

## UNITED STATES PATENT OFFICE

2,199,580

## PHOTOGRAPHIC PRINTING

Mayson H. Tucker, New York, N. Y.

No Drawing. Application September 10, 1938,  
Serial No. 229,325

6 Claims. (Cl. 95—8)

This invention relates to photographic printing and has for its principal object to provide an improved photographic printing paper capable of being printed upon in halftones, developed and fixed in white light. The invention also provides a method for carrying out photographic printing operations in white light and a method for preparing the paper of the invention.

In contact printing of photographs in halftones from picture negatives it has heretofore been practically necessary to develop and fix the exposed print in the dark, or at least in a dim light substantially free from actinic rays. While this disadvantage to heretofore known methods of photographic printing is of no particular consequence to professional photographers, it is of considerable consequence to amateurs who find it difficult to provide the necessary dark-room facilities.

Various attempts have been made to develop methods to make it possible to print photographically in ordinary white light, but such attempts have not proven particularly successful. It has been proposed, for example, to incorporate a colored dye (such as phenolphthalein) in the solutions employed for development and fixing of the photographic image after exposure of the printing paper, but this expedient still requires that the paper be mounted in the printing frame and that the exposed paper be transferred from the printing frame to the developer and from the developer to the fixing solution in the dark-room. Such procedure thus eliminates the need for a dark-room only during those phases of the printing operation when the printer has little need for light.

In accordance with the present invention, a photographic paper is provided which may be exposed to ordinary subdued daylight or artificial white light (of the order of brightness of about 10 foot-candles or less), such as ordinary indoor reading light, without becoming fogged, but which may readily be printed upon in halftones (as from a picture negative in contradistinction to photostat type of printing) by exposure to very bright light (of the order of brightness of about 500 foot-candles or more), such as the light within a fraction of an inch of the bulb of a common 60 watt electric lamp of the so-called "Mazda" type, and may be subsequently developed and fixed in ordinary indoor light without fogging.

The paper of the invention comprises a paper backing coated with a standard well-known photo-sensitive emulsion applied to a surface there-

of and having a colored dye applied as a separate film over the exposed surface of the sensitive emulsion.

The colored dye as it is employed on the film is of such character as to be substantially opaque to the actinic rays of ordinary subdued daylight or artificial white light of brightness of the order of about 10 foot-candles or less, but is capable of transmitting at least a portion of the actinic rays of very bright light of brightness of the order of about 500 foot-candles or more.

In referring to the quality of the colored dye as "substantially opaque" to the actinic rays of ordinary subdued daylight or the like and as "capable of transmitting" or "transparent to" a portion of the actinic rays of very bright light, it is of course understood that such opacity or transparency is a relative quality which can be reduced to an absolute quality only by taking into account the element of time. Thus, even a colored dye which, in the form of a film over a photo-sensitive emulsion, is "substantially opaque" to the actinic rays of a subdued light within the meaning of the term as used herein, will pass a sufficient quanta of such rays, if exposed to the subdued light for a long enough period of time, to fog the paper; and conversely, even if the dye is "capable of transmitting" a portion of the actinic rays of very bright light within the meaning of that term as herein employed, it is possible to expose the paper to such a light for so short a period of time that no perceptible effect of the exposure is to be observed. These terms are therefore employed herein in a relative sense and are to be interpreted in the light of common practice in photographic printing operations.

For example, in making a contact photographic print it is awkward to have to expose the paper to a bright light of the order of 500 foot-candles in brightness for a period of time much greater than about one minute. If much more time than this is required for a colored dye applied over the surface of a sensitive emulsion to pass sufficient actinic rays of such bright light properly to expose the emulsion, the dye film ordinarily (except in cases where extremely "slow" paper is desired) is regarded, for the purposes of the invention, as not "capable of transmitting" a sufficient portion of the actinic rays of the bright light. On the other hand, for example, the ordinary amateur printing operation requires a total time (from start of preparation for exposure to fixed print) of about five minutes or less, and if paper having its sensitive emulsion coated with a colored dye fogs appreciably upon

exposure for such a period of time (or even for ten or fifteen minutes) to subdued light of a brightness of about 10 foot-candles or less, it is ordinarily regarded as not "substantially opaque" to the actinic rays of such light. But if the dye is of such character as to protect the sensitive emulsion from fogging upon exposure of the paper to ordinary subdued indoor light for the length of time required to complete the printing 10 operation, and if the dye does permit passage of actinic rays to a sufficient extent to enable proper exposure of the paper by a bright light in a period of time reasonable for the nature of the particular printing operation, the dye is regarded as 15 having the aforementioned qualities of opacity to actinic rays of subdued white light and transparency to actinic rays of bright light, as these terms are used herein and in the appended claims.

For common black and white printing in half-tones, the dye further is of such character that, upon immersion of the paper in a solution for development or fixing of a photographic image (or upon suitable washing after development and fixing), the color imparted thereby to the surface 20 of the paper is discharged. Preferably the color of the dye is discharged upon immersion of the paper in the fixing solution, for it is desirable to continue the protection provided by the dye during immersion of the paper in the developing solution, and it is inconvenient to have to subject the paper to further treatment after completion of the fixing operation.

The dyes that have proven most satisfactory for use in accordance with the invention belong 30 generally to the class known chemically as indicators. Indicators which are suitably colored in substantially neutral and mildly alkaline solutions and colorless in weakly acid solution are especially satisfactory, for such indicators may be 35 applied in the colored state to the sensitive emulsion coating of the paper (which usually is very slightly acid) and will remain colored thereon for normal periods of storage and during immersion of the paper in the ordinary slightly alkaline developing solution. Upon subsequent immersion of 40 the paper in the conventional slightly acid fixing and hardening solution, the color of such indicator dyes will be discharged. It is not necessarily characteristic of suitable indicator dyes, however, that their color is discharged by the acidity 45 of the fixing solution. Rosolic acid, which is an especially satisfactory dye of the indicator class, appears to have its color discharged by a bleaching action of the acid sulphite fixing solution, and 50 the color of nitrophenols, which also are dyes of the indicator class, are best discharged by immersion of the paper before or after fixing, in ethyl alcohol.

A number of indicators have been employed as 55 dyes in accordance with the invention with varying degrees of success. Phenolphthalein, which in alkaline solution is pink, has been employed in the colored condition as a thin film over the photo-sensitive emulsion of a printing paper. Phenolphthalein retains its color in the usual alkaline developing solution, but upon immersion of the paper treated therewith in a standard slightly acid fixing solution the color is substantially 60 completely discharged. Phenolphthalein, however, does not provide very satisfactory protection for the sensitive emulsion even in subdued light, and its use therefore is not recommended. Its pinkish color was not sufficiently deep to exclude the damaging actinic rays of ordinary subdued white light, and, moreover, it tended to turn

colorless upon standing in contact with the sensitive emulsion. This latter disadvantage could be overcome only by considerably increasing the alkalinity of the emulsion, but this expedient so increased the speed of the emulsion that the protective character of the phenolphthalein was more than offset. For this reason it is generally undesirable to employ an indicator dye that requires an alkaline environment to maintain it in the colored state.

Ortho, meta and para nitrophenols have also been employed, and being, in neutral and mildly alkaline solutions, deep yellow to orange in color, provide good protection for the photo-sensitive emulsion. Some difficulty is apt to be experienced, however, in securing complete discharge of the color of these compounds by means of the usual weakly acidic developing or fixing solutions. Three or four minutes' immersion of paper treated with one of the nitrophenols in a slightly acid sulphite fixing solution usually is necessary to secure complete discharge of the color, and after the fixing solution has been used a number of times it acquires a yellowish color itself and to a considerable extent loses its power to discharge the color of the dye. But by dipping the paper in ethyl alcohol before or after completion of the fixing and hardening operation, the color of these dyes can be discharged quite speedily.

Picryl methyl nitrarnine, which is yellow to 30 brown in alkaline solutions and colorless in acid, is a moderately satisfactory indicator for use in accordance with the invention, but some difficulty is experienced in applying a coating of sufficient depth of color adequately to protect the film and 35 its color is somewhat difficult to discharge.

One of the most satisfactory indicators for use in accordance with the invention, is rosolic acid, which is of orange color in relatively low concentration in substantially neutral solutions, but 40 turns colorless upon immersion in the usual slightly acid sulphite or metabisulphite fixing solution, and in general the use of this compound is preferred. Its natural orange color (which is apparent with the compound in low concentration 45 in substantially neutral solutions) provides excellent protection for photo-sensitive emulsions, and the fact that its color does not depend upon the maintenance of a markedly alkaline environment makes use of this compound particularly 50 advantageous. In fact, its natural orange color provides better protection for the emulsion than does the reddish color it exhibits in alkaline solutions. Moreover, the speed with which its color 55 is discharged upon immersion in a sulphite fixing solution renders it particularly easy to employ.

The rosolic acid or other indicator or dye is applied to ordinary photographic printing paper as a separate colored film over the exposed surface of the photo-sensitive emulsion (which may be 60 any suitable emulsion such as the common silver chloride emulsion), preferably after the latter has dried on the paper, and there it appears as a colored film which substantially excludes the actinic rays of ordinary white light from the sensitive emulsion. In some cases, alternatively, the dye may be incorporated in the top hardening coating overlying the main emulsion. The amount of indicator or dye thus applied is sufficient to form a film deep enough in color to be 70 substantially opaque (as hereinbefore defined) to the actinic rays of light of brightness of the order of about 10 foot-candles, but transparent (as hereinbefore defined) to at least a portion of the actinic rays of a very bright light of the order of 75

500 foot-candles in brightness. For the ordinary photographic printing paper, coated for example, with the usual silver chloride emulsion, satisfactory protection has been obtained with dyes 5 forming a film colored a moderately deep yellow, orange, tan or light brown, or a deep red. Blue or violet colored dyes are not recommended for such paper.

In employing rosolic acid, for example, a solution of this compound in an alcoholic solvent is applied over the emulsion surface of a standard photographic paper by any suitable coating operation, as by spraying, dipping or painting, preferably after the emulsion has become substantially completely dried. The solution employed should contain at least about 2% rosolic acid in order sufficiently to color the surface of the paper, and in general it is preferred to employ a solution containing about 2½% to 3% rosolic 20 acid. Such a solution colors the surface of the paper a moderately deep orange, which substantially excludes the actinic rays of ordinary indoor light from the photosensitive emulsion.

It is important that the solution of rosolic acid 25 or other indicator or dye be applied uniformly and without the occurrence of "flutter" or unevenness of coating on the paper, for otherwise the opacity of the dye film to actinic rays will vary from point to point on the paper and it 30 will not be possible to expose the paper uniformly. In the case of rosolic acid, if it is simply dissolved in ethyl alcohol and the alcohol solution is spread on the emulsion for example, the solvent evaporates so rapidly that nonuniform coating or "flutter" 35 is apt to result. For this reason, it is preferred to apply the rosolic acid in solution in an ethyl alcohol-water solvent containing about 20% by weight of water. It is preferable to use distilled water in the alcohol-water solvent, for tap 40 water commonly is alkaline enough to convert the color of the rosolic acid from its natural orange to the less desirable red. While it is possible to use a solvent containing considerably more than 20% and up to 61% water (above this latter concentration of water the rosolic acid 45 tends to precipitate), the use of such high water concentration in the solvent leads to difficulties in securing substantially complete color-discharge in the fixing bath. It is also advantageous 50 ordinarily to incorporate in the solution a non-hygroscopic material capable of retarding the rate of evaporation of the solution, such as a small percentage of the order of 1% by weight of the solvent of a sugar or sugar-like compound. 55 Very satisfactory results have been obtained using rosolic acid dissolved in a solvent employing ethyl alcohol and water in equal parts by weight and containing about 0.75% by weight of a product available under the trade name "Yumidol Special," which is a colorless refined, water 60 solution containing about 85% sorbitol (a sugar-like, hexahydric alcohol), and which is a viscous, non-hygroscopic, colorless liquid, soluble to the extent necessary both in alcohol and water. 65 Fructose and other similar materials may also be employed, but the use of glycerine, ethylene glycol and the like is excluded because these materials are so hygroscopic that they are apt to render the emulsion tacky and cause injury 70 thereto if applied thereto.

Paper prepared in accordance with the invention is employed by first exposing it in a contact printing frame to a very bright light of brightness of the order of 500 foot-candles. For this purpose, use of the photographic printing method

and apparatus defined in my copending application Serial No. 232,045, filed September 28, 1938, is especially satisfactory. Although it is possible under special conditions to print on the paper of the invention at a distance, an extremely intense light or a well-focused one is required, and this practice is not recommended to the amateur. Even in making contact prints it is important that the paper be held close to the source of light and that the distribution of light over 10 its surface be uniform in order that it may be properly exposed.

After exposure, the paper is immersed in a developing solution for purposes of development of the photographic image formed by the exposure. Any of the standard well-known developing solutions suitable for the type of emulsion used on the paper may be employed. One such developing solution that has been employed with success is a compound consisting of about 3.1 20 grams "Elon" (a well-known developing reagent manufactured by the Eastman Kodak Co.), about 45 grams hydroquinone, about 67.5 grams sodium carbonate, about 1.9 grams potassium bromide, and about 45 grams sodium sulphite dissolved to 25 one liter in water.

When rosolic acid is employed as the dye on the surface of the emulsion (as is preferred) it is desirable to incorporate a colored agent, such as phenolphthalein, in the developer for the purpose of excluding actinic rays therefrom. Rosolic acid turns to a red color in the standard alkaline developing solutions, and when this color it does not provide as complete protection against fogging as it does when orange in color. 30

After immersion of the paper in the developer for a suitable period of time, it is transferred to a fixing bath in which the developed photographic image is fixed and in which, preferably, the color of the dye is discharged. Any standard fixing bath may be employed, such as the well-known water solution of about 480 grams sodium thiosulphate (hypo), about 30 grams sodium sulphite or sodium metabisulphite, about 30 grams alum, and about 96 cc. of 28% acetic acid dissolved in about 2160 cc. of water. In the preferred application of the invention employing rosolic acid as the dye, the color of the rosolic acid is quickly discharged in such a fixing bath and a clear black and white print is obtained. All of these printing operations may be carried out in a subdued light of the order of about 10 40 foot-candles in brightness. 45

Rosolic acid generally is noted as turning from red in alkaline solution to yellow or yellow brown in acid, but in the fixing solution its color is substantially completely discharged. It therefore appears that a bleaching action of the sulphite dissolved in the fixing bath is, at least in part, responsible for the color change. The acid of the bath seems to play some part in this change, however, for in the alkaline developing bath, which also usually contains some sodium sulphite, the color is changed only to a red, and is not completely discharged. 50

In the foregoing specification and in the claims particular reference is made to photographic printing "paper" having a "paper" backing. Most photographic "paper" does in fact have a backing of paper, but in some cases a backing 55 of some other flexible material is employed. It is understood that the process of the invention is fully applicable to products backed with such other flexible material (as Celluloid or cellulose acetate film) as it may be desired to employ. If 60 65 70 75

the backing is transparent, the dye used is applied in a manner to protect the emulsion from light on both sides thereof, as by applying it to the back of the backing as well as over the exposed surface of the emulsion. Otherwise no substantial departure need be made from the procedure set forth above.

I claim:

1. A photographic printing paper adapted to be printed upon, developed and fixed in white light, comprising a paper backing, a coating of a photo-sensitive emulsion applied to a surface of said backing, and rosolic acid in its colored state applied as a separate film over the exposed surface of said emulsion, said colored rosolic acid film being of such a depth of color as to permit exposure of the emulsion-coated surface of the paper at least for a short period of time to subdued white light with fogging, but being sufficiently transparent to the actinic rays of very bright light to enable formation on the light-sensitive emulsion of a photographic image by exposure of the dye-coated surface of the paper to a bright light.
2. A photographic printing paper adapted to be printed upon in half-tones, developed and fixed in white light, comprising a substantially opaque paper backing, a coating of a photo-sensitive emulsion applied to a surface of said backing, and rosolic acid in its colored state applied as a separate film over the exposed surface of said emulsion, said rosolic acid film being sufficiently deep in color to be substantially opaque to the actinic rays of subdued daylight or artificial white light of brightness of the order of about 10 foot-candles, but being capable of transmitting at least a sufficient amount of the actinic rays of very bright light of brightness of the order of 500 foot-candles to enable formation on the emulsion of a photographic image, whereby the emulsion-coated surface of said paper may be exposed at least for a short period of time to subdued white light without fogging, but may be printed upon by exposure of its dye-coated surface to a bright light.
3. In printing photographically on a photographic paper comprising a photo-sensitive emulsion on a suitable backing, the improvement which comprises enabling printing in half-tones, developing and fixing in ordinary subdued daylight or artificial white light of a photographic image on said paper by applying to the exposed surface of the photo-sensitive emulsion a separate film of rosolic acid in its colored state, said rosolic acid film being applied to such a depth of color as to be substantially opaque to the actinic rays of subdued light of brightness of the order of about 10 foot-candles but capable of transmitting at least a sufficient amount of the actinic rays of very bright light of brightness of the order of 500 foot-candles to enable formation on the emulsion of a photographic image, exposing the rosolic acid coated surface of said paper in contact with a suitable negative to a very bright light, immersing the exposed paper in a suitable developing solution to develop the photo-

tographic image thereon, and subsequently immersing the paper in an acidic sulphite fixing solution in a manner such that the developed photographic image thereon is fixed and the color of the rosolic acid is substantially completely discharged.

4. In printing photographically on a photographic paper comprising a photo-sensitive emulsion on a suitable backing, the improvement which comprises enabling printing in half-tones, developing and fixing in ordinary daylight or artificial white light of a photographic image on said paper by applying to the exposed surface of the photo-sensitive emulsion a separate film of rosolic acid in its colored state, said rosolic acid film being applied to such a depth of color as to be substantially opaque to the actinic rays of subdued light of brightness of the order of about 10 foot-candles but capable of transmitting at least a sufficient amount of the actinic rays of very bright light of brightness of the order of 500 foot-candles to enable formation on the emulsion of a photographic image, exposing the rosolic acid coated surface of said paper in contact with a suitable negative to a very bright light, thereafter immersing said paper in a developing solution containing a dye of such color and in such concentration that actinic rays of ordinary daylight or artificial white light are substantially excluded from said solution, and subsequently immersing said paper in an acidic sulphite fixing solution in a manner such that the developed photographic image thereon is fixed and the color of the rosolic acid is substantially completely discharged.

5. In the preparation of a photographic printing paper comprising a backing, a photo-sensitive emulsion applied to a surface of said backing, and rosolic acid applied in a colored state as a separate film over the exposed surface of said emulsion, the method of forming said rosolic acid film evenly and uniformly on said emulsion which comprises dissolving rosolic acid in a solvent comprising about 80% ethyl alcohol and about 20% water by weight, and suitably coating the resulting solution over the exposed emulsion surface of the emulsion-coated paper after the emulsion has become substantially completely dried.

6. In the preparation of a photographic printing paper comprising a backing, a photo-sensitive emulsion applied to a surface of said backing, and rosolic acid applied in its colored condition as a separate film over the exposed surface of said emulsion, the method of forming said rosolic acid film evenly and uniformly on said emulsion which comprises dissolving the rosolic acid in a solvent comprising about 20% by weight of water and about 80% by weight of ethyl alcohol and a small percentage of the order of 1% of a non-hygroscopic sugar, and suitably coating the resulting solution on the emulsion surface of the emulsion-coated paper after the emulsion has become substantially completely dried.

MAYSON H. TUCKER.